# EUROPEAN PATENT SPECIFICATION

(11) **EP 1 471 137 B1**
(45) Date of publication and mention of the grant of the patent: **07.08.2013**
(21) Application number: 03252549.5
(22) Date of filing: 23.04.2003
(51) Int. Cl.: C11D 17/00, C11D 3/50, C11D 3/37

(54) **A composition comprising a surface deposition enhacing cationic polymer**
Zusammensetzung enthaltend ein kationisches Polymer zur verbesserten Abscheidung an einer Oberfläche
Composition comprenant un polymere cationique ameliorant la deposition en surface

(43) Date of publication of application: 27.10.2004
(73) Proprietor: THE PROCTER & GAMBLE COMPANY, Cincinnati, OH 45202 (US)
(72) Inventor: Meli, Fabrizio, Tynemouth, Tyne & Wear NE30 4BE (GB); Chieffi, Andre, Tynemouth, Tyne & Wear NE30 4JX (GB)
(74) Representative: Howard, Phillip Jan

(56) References cited:
- EP-A- 0 523 287
- WO-A-01/40430
- WO-A-94/28107
- WO-A-97/48375
- US-A- 3 761 418
- US-A- 4 536 315
- US-B1- 6 221 826

## Description

### Technical Field

The present invention relates to detergent auxiliary compositions in particulate form comprising a surface deposition enhancing cationic polymer, methods of making said detergent auxiliary compositions, laundry detergent compositions comprising said detergent auxiliary compositions and use of said surface deposition enhancing cationic polymer to enhance the deposition of a perfume onto a fabric surface.

### Background to the invention

Surface treatment compositions, such as fabric treatment compositions including laundry detergent compositions, typically comprise systems that deposit actives onto the surface to be treated. For example, laundry detergent compositions may comprise active components that need to be deposited onto the fabric surface before they can carry out their intended action. These active components include perfumes.

However, laundry detergent compositions are typically designed to remove material, i.e. soil, from the surface of a fabric during a laundering process. Therefore, the majority of the chemistry that is formulated into a laundry detergent composition is designed and tailored to carry out this task. Thus, it is difficult to deposit any active component onto a fabric surface during a laundering process due to this chemistry. This problem is especially true for active components that are liquid or liquefiable, such as perfumes, which are particularly troublesome to deposit onto a fabric surface during a laundering process.

Attempts have been made to improve the deposition of perfume onto a fabric surface during a laundering process by using hydrophobic perfume raw materials that have high boiling points; thus not readily evaporating from the wash liquor and more readily associating with the fabric surface due to having an increased hydrophobic interaction with the fabric surface. These perfumes are known as quadrant 4 perfume raw materials and are described in more detail in US5500138 and US6491728. However, the disadvantage of using quadrant 4 perfumes in laundry detergent compositions is that the perfumer is very limited in the choice of perfume raw materials that he can use, and the odours these quadrant 4 perfumes deliver are very musky odours that are not always suitable for use in laundry detergent compositions. In addition, the deposition of quadrant 4 perfumes onto the surface of a fabric during a laundering process is still not very efficient and still needs to be improved.

Other attempts to improve the fabric surface deposition of perfumes during a laundering process include the encapsulation of perfume raw materials, for example in starch to obtain a starch-encapsulated perfume accord. These starch-encapsulated perfume accords and their applications in laundry detergent compositions are described in more detail in WO99/55819 However, these starch-encapsulated perfume accords, although giving good wet stage odour benefits, are not designed to give optimal deposition of perfume onto the surface of a fabric during a laundering process, presumably being due to the fact that they are readily water-soluble and/or water-dispersible in the wash liquor and the majority of the perfume is lost in the wash liquor during the laundering process. Thus, there is a need to improve the deposition of perfume onto a fabric surface during a laundering process.

Another approach is the loading of perfume onto porous carrier materials such as zeolite. This perfume-loaded zeolite approach is described in more detail in EP701600, EP851910, EP888430, EP888431, EP931130, EP970179, EP996703, US5691383, US5955419 and WO01/40430. However, there is a risk that the perfume may leak from the zeolite onto the detergent matrix during storage and/or leak into the wash liquor (i.e. before the zeolite has been deposited onto a fabric surface) during a laundering process. In order to overcome this problem, attempts have also been made to encapsulate these perfume-loaded zeolites with starch; this is described in more detail in EP859828, EP1160311 and US5955419. However, there is still a need to further improve the deposition of perfume onto the surface of a fabric during a laundering process.

There still remains a need to further improve the deposition of liquid or liquefiable active components such as perfume onto a fabric surface during a laundering process. The inventors have surprisingly found when a cationic polymer is incorporated into a detergent auxiliary composition in particulate form that comprises a solid support component, an active component and an encapsulating material, the surface deposition of the active component is improved. The inventors have also surprisingly found that when the cationic polymer is of a specific highly preferred weight average molecular weight or has a specific highly preferred average degree of cationic substitution or both, then the surface deposition of the active component is improved whilst avoiding cleaning negatives.

US 4536315 relates to compositions comprising perfume and zeolite.

### Summary of the invention

The present invention provides a detergent auxiliary composition in particulate form, comprising: (i) a liquid or liquefiable active component; and (ii) a water-insoluble solid support component and (iii) a water-soluble and/or water dispersible encapsulating material; and (iv) optionally one or more adjunct components, characterised in that the composition further comprises (v) a surface deposition enhancing cationic polymer, wherein the cationic polymer is adsorbed onto the solid support component, and wherein the encapsulating material encapsulates the active component, the solid support component and the cationic polymer.

### Detailed description of the invention

### Detergent auxiliary composition in particulate form

The detergent auxiliary composition is suitable for incorporation into a detergent composition, such as a laundry detergent composition; i.e. to make a fully formulated detergent composition. Alternatively, the detergent auxiliary composition is suitable for use in combination with a detergent composition such as a laundry detergent composition: i.e. as an additive to an already fully formulated detergent composition. The detergent auxiliary composition is in particulate form and comprises a liquid or liquefiable active component, a water-insoluble solid support component, a water-soluble and/or water dispersible encapsulating material, a surface deposition enhancing cationic polymer and optionally one or more adjunct components. All of these are discussed in more detail below.

Since the composition is designed to deposit the active component onto the treated surface, the particle should be capable of coming into close proximity with the treated surface. One means of achieving this is to ensure that there is little or no repulsion between the particles of the composition and the treated surface, i.e. little or no electrochemical repulsion. It is therefore desirable to keep the electrokinetic potential, also known as the zeta potential, of the composition low in order to minimize any electrochemical repulsion that may occur between the composition and the treated surface. Zeta potential is described in more detail in the Physical Chemistry of Surfaces, 4th Edition, 1982, written by Adamson and published by John Wiley & Sons, especially pages 198-205 of the above document.

The zeta potential of the composition is typically determined by the following method:
1. Add 10g of composition to 200ml of water at 25°C and agitate for 5 minutes.
2. Centrifuge the product of step 1 for 8,000rpm for 10mins in a Sigma 4-10 centrifuge.
3. Separate the sediment collected during step 2 and suspend 0.02g of the sediment in 500ml of an aqueous solution of 1mM KCl.
4. Fill the chamber of a Brookhaven ZetaPlus Zeta Potential Analyzer with the above suspension of step 3.
5. Insert the full chamber into the analyser and analyse the zeta potential according the manufacturer's instructions.
6. Take an average of 10 readings to determine the zeta potential of the composition.

Preferably, the composition has a zeta potential that is more neutral than -30mV, preferably more neutral than -20mV. It is believed that the lower (i.e. more neutral) zeta potential is achieved due to the presence of the surface deposition enhancing cationic polymer in the composition. The composition preferably comprises from 1.2wt% to 10wt% surface deposition enhancing cationic polymer.

The composition typically has a mean particle size of from 5 micrometers to 200 micrometers, preferably from 10 to 50 micrometers, and/or typically no more than 10wt% of the composition has a particle size less than 5 micrometers and/or typically no more than 10wt% of the composition has a particle size greater than 80 micrometers. These particle size requirements and distributions are especially preferred when the detergent auxiliary composition is incorporated in a laundry detergent composition, as particles having these particle size requirements and distributions do not segregate in the laundry detergent composition during transport and storage, and are stable in the laundry detergent composition during storage.

The composition may be obtainable, and/or may be obtained, by an agglomeration, spray-drying, freeze-drying or extrusion process. However, there is a highly preferred order in which the components that make up the composition are contacted to each other during the process of making the composition. This preferred process is described in more detail below.

### Active component

The active component is in a liquid or liquefiable form. Preferably the active component is in liquid form. The active component typically needs to be brought into close proximity with or even deposited onto the treated surface during the treatment process before it can carry out its intended function. An active component is any component for which there is a need and/or requirement to deposit it onto the treated surface, for example, to enhance its performance. The active components are not limited to active components that are inactive until they are in close proximity to, or deposited onto, the treated surface. A highly preferred active component is perfume, especially when it is desired to deliver a good dry fabric odour benefit to a fabric during a laundering process.

The perfume can be formulated to provide any olfactory perception that is desired. For example, the perfume can be a light floral fragrance a fruity fragrance or a woody or earthy fragrance. The perfume typically comprises one or more perfume raw materials (PRMs), more typically the perfume comprises numerous PRMs, i.e. at least two, or at least five or even at least ten and typically even more than that, which are typically blended together to obtain a perfume that has the desired odour. The perfume may be of a simple design and comprise only a relatively small number of PRMs, or alternatively the perfume may be of a more complex design and comprise a relatively large number of PRMs. Suitable PRMs are typically selected from the group consisting of aldehydes, ketones, esters, alcohols, propionates, salicylates, ethers and combinations thereof. Preferred perfumes and PRMs are described in more detail in WO97/11151, especially from page 8, line 18 to page 11, line 25.

The perfume typically has a threshold olfactory detection level, otherwise known as an odour detection threshold (ODT) of less than or equal to 3ppm, more preferably equal to or less than 10ppb. Typically, the perfume comprises PRMs that have an ODT of less than or equal to 3ppm, more preferably equal to or less than 10ppb. Preferred is when the perfume comprises at least 70wt%, more preferably at least 85wt%, PRMs that have an ODT of less than or equal to 3ppm, more preferably equal to or less than 10ppb. A method of calculating ODT is described in WO97/11151, especially from page 12, line 10 to page 13, line 4. Typically, the perfume has a boiling point of less than 300°C. Typically, the perfume comprises at least 50wt%, more preferably at least 75wt%, of PRMs that have a boiling point of less than 300°C. In addition, the perfume typically has an octanol/water partition coefficient (ClogP) value greater than 1.0. A method of calculating ClogP is described in WO97/11151, especially from page 11, line 27 to page 12, line 8.

The active component, or at least part thereof, is typically adsorbed and/or absorbed onto the solid support component. This is especially preferred when the solid support component is porous and the active component (or if the active component is a perfume, then the PRMs that make up the perfume), or part thereof, can pass through the pores of the porous solid support component and be held within the porous matrix of the solid support component. Active components, especially perfumes, that are adsorbed/absorbed onto the porous solid support component can be tailored in such a way to delay the release of the active component from the solid support component.

One means of tailoring a perfume to be released slowly from a porous material is to ensure that the perfume comprises one or more PRMs that have good affinity for the porous material. For example, PRMs that have a specific size, shape (i.e. a molecular cross-sectional area and molecular volume) and surface area relative to the pores of the porous material, exhibit improved affinity for the porous material and are capable of preventing other PRMs that have less affinity to the porous material from leaving the porous material during the washing and/or rinsing stage of a laundering process. This is described in more detail in WO97/11152, especially from page 7, line 26 to page 8, line 17.

Another means of tailoring a perfume to be released slowly from a porous material is to ensure that the perfume comprises PRMs that are small enough to pass through the pores of the porous material, and that are capable of reacting together, or with a small non-perfume molecule (otherwise known as a size-enlarging agent) to form a larger molecule (otherwise known as a release inhibitor) that is too large to pass through the pores of the porous material. The release inhibitor, being too large to pass through the pores of the porous material, becomes entrapped within the porous matrix of the porous material until it breaks down (i.e. hydrolyses) and reverts back to the smaller PRM and size enlarging agent, which are then capable of passing through the pores of, and exiting, the porous material. Typically, this is achieved by the formation of hydrolysable bonds between a small PRM and a size-enlarging agent, to form a release inhibitor within the porous material. Upon hydrolysis, the small PRM is released from the larger molecule and is then capable of exiting the porous material. This is described in more detail in WO97/34981, especially from page 7, line 4 to page 5, line 14.

In addition, the above approach of forming a release inhibitor by reacting a PRM with a size-enlarging agent can be further adapted by using a size enlarging agent that has a hydrophilic portion and a hydrophobic portion (e.g. a sugar based non-ionic surfactant such as a lactic acid ester of a C₁₈ monoglyceride). This is described in more detail in WO97/34982, especially from page 6, line 27 to page 7, line 17.

### Solid support component

The solid support component is insoluble in water. The solid support component interacts with the active component to provide a support for and to protect the active component during a treatment process such as a laundering process. The solid support component also enhances the deposition of the active component onto a treated surface, e.g. a fabric surface, typically by being deposited onto the treated surface itself and carrying the active component onto the treated surface with it.

The solid support component can be any water-insoluble material that is capable of supporting (e.g. by absorption or adsorption) the active component, whilst, of course, still being able to release the active component at some stage during and/or after the treatment process. Preferred solid support components are porous materials, such that the active component can pass through the pores of the porous solid support component and be held within the porous matrix of the solid support component.

Preferred solid support components are selected from the group consisting of aluminosilicates, amorphous silicates, calcium carbonates and double salts thereof, clays, chitin micro beads, crystalline non-layered silicates, cyclodextrins and combinations thereof. More preferably, the solid support component is an aluminosilicate, most preferably a zeolite, especially a faujustite zeolite, such as zeolite X, zeolite Y and combinations thereof. An especially preferred solid support component is zeolite 13x. Preferred aluminosilicates are described in more detail in WO97/11151, especially from page 13, line 26 to page 15, line 2.

It may be preferred for the solid support component to have a crystalline structure and to have an average primary crystal size in the range of from 2 to 80 micrometers, preferably from 2 to 10 micrometers and/or typically no more than 10wt% of the primary crystals have a particle size less than 0.8 micrometers and/or typically no more than 10wt% of the primary crystals have a particle size greater than 20 micrometers. Solid support components having these primary crystal size requirements show good deposition onto the treated surface, show good release dynamics of the active component, show improved active component loading capability and do not give rise to any cleaning and/or treatment negatives.

Preferably, the outer surface of the solid support component has a negatively charged surface, especially when at neutral pH (i.e. pH 7). Typically, the solid support component comprises an oxide outer surface; i.e. the outer surface of the solid support component comprises oxide moieties. A solid support component having a negatively charged outer surface charge, more readily interacts with the surface deposition enhancing cationic polymer, due to increased electrochemical attraction between the cationic polymer and negatively charged outer surface of the solid support component. This is especially preferred when the surface deposition enhancing cationic polymer has a specific charge density and/or a specific degree of cationic substitution, as then there is an optimal affinity between the cationic polymer and the solid support component, which results in improved deposition of the active component onto the treated surface, especially a fabric surface during a laundering process.

### Encapsulating material

The encapsulating material is water-soluble. The encapsulating material encapsulates all of the active component, solid support component and cationic polymer. In this manner, the encapsulating material protects the components it encapsulates from the external environment during storage and also during the early and possibly even late stages of the treatment process. The encapsulating material typically dissolves at some point during the washing stage of the treatment process, and releases the solid support component along with the active component and surface deposition enhancing cationic polymer, into the wash liquor. The solid support component is then able to deposit onto the treated surface and bring the active component into close proximity to the treated surface.

The encapsulating material can be used as a delay release means for the active component in the treatment process. For example, the water-solubility of the encapsulating material can be increased or decreased to enable the release of the active component into the wash liquor at an early or late stage in the treatment process. For example, if the active component is a perfume and it is desired to deliver a good dry fabric odour benefit to a fabric during a laundering process, then it may be preferred to delay the release of the perfume into the wash liquor until a late stage in the laundering process so as to prevent, or greatly reduce, the loss of perfume which may otherwise occur.

The encapsulating material may have a glass transition temperature (Tg) of 0°C or higher. Glass transition temperature is described in more detail in WO97/11151, especially from page 6, line 25 to page 7, line 2. By controlling the glass transition temperature of the encapsulating material, the frangibility of the composition can be controlled to avoid the break up of the composition, which is in particulate form, during handling, transport and storage, this will also reduce the generation of dust which may occur during handling and transport. One way to control the glass transition temperature of the encapsulating material is to incorporate a plasticiser, typically, a plasticiser other than water, in the encapsulating material. Any known plasticisers, other than water, can be used. If the encapsulating material is a starch, then preferred plasticisers are selected from the group consisting of mono- and di-saccharides, glycerine, polyols and mixtures thereof

The encapsulating material is preferably selected from the group consisting of carbohydrates, natural and/or synthetic gums, cellulose and/or cellulose derivatives, polyvinyl alcohol, polyethylene glycol, and combinations thereof. Preferably the encapsulating material is a carbohydrate, typically selected from the group consisting of monosaccharides, oligosaccharides, polysaccharides, and combinations thereof. Most preferably, the encapsulating material is a starch. Preferred starches are described in EP922499, US4977252, US5354559 and US5935826.

### Surface deposition enhancing cationic polymer

The surface deposition enhancing cationic polymer enhances the deposition of the active component, which is usually held within or by the solid support component, onto the surface to be treated. Without wishing to be bound by theory, it is believed that the cationic polymer, once adsorbed onto the solid support component, diminishes, preferably negates, any repulsion, i.e. electrostatic repulsion, that may occur between the outer surface of the solid support component and the treated surface; this is believed to be especially true when the outer surface of the solid support component is negatively charged and the treated surface is a fabric surface. The surface deposition enhancing cationic polymer typically reduces the zeta potential of the composition.

Surface deposition enhancing cationic polymers having a highly preferred average degree of cationic substitution more readily interact with the solid support component and further enhance the deposition of the active component onto the treated surface during the treatment process. This is especially true for laundering processes and also when the active component is a perfume. The cationic polymer preferably has an average degree of cationic substitution of from 1% to 70%, preferably from above 20% to 70%, more preferably from 40% to 60%.

The average degree of cationic substitution typically means the molar percentage of monomers in the cationic polymer that are cationically substituted. The average degree of cationic substitution can be determined by any known methods, such as colloid titration. One such colloid titration method is described in more detail by Horn, D., in Prog. Colloid &Polymer Sci., 1978, 8, p243-265.

Whilst it is desirable for the cationic polymer to be able to (i) reduce the zeta potential of the composition, (ii) increase the hydrophobicity of the composition and (iii) increase the area of contact between the treated surface and the composition, as this promotes deposition of the solid component and/or active component onto the treated surface, it is also desirable that coacervation and flocculation involving the cationic polymer and other components of the composition and/or soil present in the wash liquor do not occur as this can give rise to cleaning negatives. The ability of the cationic polymer to provide the above benefits whilst avoiding coacervation and flocculation can be controlled by controlling the weight average molecular weight of the cationic polymer and the average degree of cationic substitution of the cationic polymer. It is also desirable that the cationic polymer remains adsorbed on the solid support component during the treatment process as any cationic polymer that does not remain adsorbed on the solid support component, i.e. cationic polymer that becomes free in the wash liquor, is capable of interacting with components of the composition and/or soil and can cause cleaning negatives.

If the molecular weight of the cationic polymer is too great, then the cationic polymer may promote flocculation and cleaning negatives may be observed. If the molecular weight of the cationic polymer is too small, then the deposition of the active component onto the treated surface is not optimal. Preferred cationic polymers have a weight average molecular weight of from above 100,000 Da. to below 10,000,000 Da., preferably from 500,000 Da. to 2,000,000 Da..

Any known gel permeation chromatography (GPC) measurement methods for determining the weight average molecular weight of a polymer can be used to measure the weight average molecular weight of the cationic polymer. GPC measurements are described in more detail in Polymer Analysis by Stuart, B. H., p108-112, published by John Wiley & Sons Ltd, UK, © 2002.

A typical GPC method for determining the weight average molecular weight of a polymer is described below:
1. Dissolve 1.5g of polymer in 1 litre of deionised water.
2. Filter the mixture obtained in step 1., using a Sartorius Minisart RC25 filter.
3. According the manufacturer's instructions, inject 100 litres of the mixture obtained in step 2., on a GPC machine that is fitted with a Suprema MAX (8mm by 30cm) column operating at 35°C and a ERC7510 detector, with 0.2M aqueous solution of acetic acid and potassium chloride solution being used as an elution solvent at a flux of 0.8 ml/min.
4. The weight average molecular weight is obtained by analysing the data from the GPC according to the manufacturer's instructions.

Cationic polymers having this preferred weight average molecular weight and preferred average degree of cationic substitution can be used to enhance the deposition of a perfume onto a fabric surface.

The cationic polymer is typically water-soluble and/or water-dispersible, preferably water-soluble. Water-soluble and/or water dispersible cationic polymers, especially water-soluble cationic polymers show a surprising good ability to deposit the active component onto the treated surface.

Preferred cationic polymers comprise (i) acrylamide monomer units, (ii) other cationic monomer units and (iii) optionally, other monomer units. Suitable surface deposition enhancing cationic polymers are cationically modified polyacrylamides or copolymers thereof; any cationic modification can in theory be used for these polyacrylamides. Highly preferred cationic polymers are co polymers of acrylamide and a methyl chloride quaternary salt of dimethylaminoethyl acrylate (DMA3-MeCI), for example such as those supplied by BASF, Ludwigshafen, Germany, under the tradename Sedipur CL343.

The general structure for DMA3MeCl is:

The general structure of acrylamide is:

Preferred cationic polymers have the following general structure: wherein n and m independently are numbers in the range of from 100 to 100,000, preferably from 800 to 3400. The molar ratio of n:m is preferably in the range of from 4:1 to 3:7, preferably from 3:2 to 2:3.

Suitable cationic polymers are described in more detail in, and can be synthesized according to the methods described in, DE10027634, DE10027636, DE10027638, US6111056, US6147183, WO98/17762, WO98/21301, WO01/05872 and, WO01/05874.

### Laundry detergent compositions comprising the detergent auxiliary composition

The detergent auxiliary composition is preferably incorporated in a laundry detergent composition. The laundry detergent composition is used to launder fabrics and provides a good dry fabric odour benefit to the fabric due to the presence of the detergent auxiliary composition in the laundry detergent composition. The laundry detergent composition typically comprises one or more adjunct components. These adjunct components are described in more detail below. The laundry detergent composition may be the product of a spray-dry and/or agglomeration process.

### Optional adjunct components

The detergent auxiliary composition and/or the laundry detergent composition may optionally comprise one or more adjunct components. These adjunct components are typically selected from the group consisting of detersive surfactants, builders, polymeric co-builders, bleach, chelants, enzymes, anti-redeposition polymers, soil-release polymers, polymeric soil-dispersing and/or soil-suspending agents, dye-transfer inhibitors, fabric-integrity agents, brighteners, suds suppressors, fabric-softeners, flocculants, and combinations thereof. Suitable adjunct components are described in more detail in WO97/11151, especially from page 15, line 31 to page 50, line 4.

### Method of making the detergent auxiliary composition

The detergent auxiliary composition is typically obtained by a method comprising the steps of: (i) contacting a water-insoluble solid support component with a liquid or liquefiable active component to form a first mixture; and (ii) contacting the first mixture obtained in step (i) with a surface deposition enhancing cationic polymer to form a second mixture; and (iii) contacting the second mixture obtained in step (ii) with a water-soluble and/or water-dispersible encapsulating material to form a composition; and (iv) optionally, drying the composition, wherein step (ii) occurs subsequent to step (i) and prior to steps (iii) and (iv).

Step (i) of contacting a solid support component with an active component to form a first mixture is typically carried out in a high shear mixer such as a Schuggi mixer or other high shear mixer, for example a CB mixer, although other lower shear mixers, such as a KM mixer, may also be used. Typically, the solid support component is passed through the mixer and the active component is sprayed onto the solid support component. If the active component adsorbs or absorbs onto the solid support component, which is the case if the active component is a perfume and the solid support component is a zeolite, then this reaction is typically exothermic and heat is generated during this stage of the process. This of course depends on the active component used and the solid support component used. Furthermore, the build up of heat during this step is more likely to occur when the process is a continuous process (as opposed to a batch process). The generation of heat can be controlled by any suitable heat management means; such as placing water jackets or coils on the mixer or other vessel used in step (i), or by direct cooling, for example by using liquid nitrogen, to remove the heat that is generated, and/or by controlling the flow rate of the active component and/or the solid support component in the mixer or other vessel used in step (i).

Step (ii) of contacting the first mixture obtained in step (i) with a surface deposition enhancing cationic polymer to form a second mixture can occur in any suitable vessel such as a stirred tank. Alternatively, step (ii) can occur in an online mixer. The stirred tank can be a batch tank or a continuous tank. Typically this step is carried out in an aqueous environment. Typically, the cationic polymer is diluted in water to form an aqueous mixture and to this aqueous mixture is added the first mixture obtained in step (i). The concentration of the cationic polymer in the aqueous mixture is from 0.3g/l to 50g/l, preferably from 10g/l to 30g/l. Cationic polymers being present at these preferred concentrations show optimal adsorption onto the solid support component.

In addition to this, it is also desirable to control the concentration of the solid support component in the aqueous mixture. Preferably, the concentration of the solid support component in the aqueous mixture is from 7g/l to 2,000g/l, preferably from 500g/l to 1,000 g/l. Solid components being present at these preferred concentrations enable an efficient particle production process and efficient uptake of the cationic polymer.

It may also be desirable to control the electrochemistry of the cationic polymer and the solid support component during step (ii) to ensure that they have optimal affinity to each other during this step. One means of controlling the electrochemistry is to control the pH of step (ii). Preferably step (ii) is carried out in an aqueous environment having a pH of from 3 to 9, most preferably from 4 to 7.

The time of step (ii) should typically be sufficient to allow adsorption of the cationic polymer onto the solid support material. Preferably the time of step (ii) is from 5 minutes to 25 minutes, most preferably from 10 minutes to 15 minutes.

Step (iii), of contacting the second mixture obtained in step (ii) with a water-soluble and/or water-dispersible encapsulating material to form a composition, can occur in any suitable vessel such as a stirred tank. Alternatively, step (iii) can occur in an online mixer. The stirred tank can be a batch tank or a continuous tank. It may be preferred to control the temperature of step (iii) especially in order to obtain a composition comprising a high level of active component.

Preferably, step (ii) and/or (iii) is carried out a temperature of less than 50°C, or even less than 20°C. It may be preferred that cooling means such as a water jacket or even liquid nitrogen are used in step (ii) and/or (iii), this is especially typical when it is desirable to carry out step (ii) and/or (iii) at a temperature that is below the ambient temperature. It may also be preferred to limit the energy condition of step (ii) and/or (iii) in order to obtain a composition comprising a high level of active component.

Step (ii) and/or (iii) is preferably done in a low shear mixer, for example a stirred tank. This is especially preferred if the active component is a perfume.

Optional step (iv), of drying the composition of step (iii), can be carried out in any suitable drying equipment such a spray-dryer and/or fluid bed dryer. Typically, the composition of step (iii) is forced dried (for example, spray-dried or fluid bed dried) and is not left to dry by evaporation at ambient conditions. Typically, heat is applied during this drying step. Typically, the product of step (iii) is spray-dried. If the active component is volatile, e.g. a perfume, then preferably, the temperature of the drying step is carefully controlled to prevent the active component from vapourising and escaping from the composition obtained in step (iii). Preferably, the composition of step (iii) is spray-dried in a spray-drying tower, and preferably the difference between the inlet air temperature and the outlet air temperature in the spray-drying tower is less than 100°C. This is a smaller temperature difference than is conventionally used, for example in spray-drying laundry detergent components, but is preferred in order to prevent the unwanted vapourisation of any volatile active component from the composition that was obtained in step (iii). Typically, the inlet air temperature of the spray-drying tower is from 170°C to 220°C, and the outlet air temperature of the spray-drying tower is from 90°C to 110°C. Highly preferred is when the inlet air temperature of the spray-drying tower is from 170°C to 180°C, and the outlet air temperature of the spray-drying tower is from 100°C to 105°C. It is also important that a good degree of atomisation of the composition obtained in step (iii) is achieved during the spray-drying process, as this ensures that the resultant detergent auxiliary composition has the optimal particle size distribution, having good flowability, solubility, stability and performance. The degree of atomisation can be controlled by carefully controlling the tip speed of the rotary atomiser in the spray-drying tower. Preferably, the rotary atomiser has a tip speed of from 100ms⁻¹ to 500ms⁻¹.

It may be preferred that during its processing and storage thereafter, the composition and any intermediate composition/product that is formed during its processing, is kept in an environment having a low relative humidity. Preferably the air in contact with the composition (or intermediate composition/product thereof) is equal to or lower than, preferably lower than, the equilibrium relative humidity of the composition (or intermediate composition/product thereof). This can be achieved, for example, by placing the composition in air tight containers during storage and/or transport, or by the input of dry and/or conditioned air into the mixing vessels, storage and/or transport containers during the process, transport and/or storage of the composition (or intermediate composition/product thereof).

### Examples

### Example 1 - Synthesis of a copolymer of acrylamide and DMA3MeCl (1:1 ratio)

In a 2000 ml polymerisation vessel, equipped with an agitator, a condenser, a nitrogen gas inlet and inlets for addition of ingredients, the following ingredients are mixed:
(i) 882 g water; and
(ii) 0.15 g Trilon C (premixed in water at a concentration of 40w/v%).
This mixture is then heated to a temperature of 75°C, after which,
(iii) 255.95 g DMA3MeCl (methyl chloride quaternary salt of dimethylaminoethyl acrylate) (premixed in water at a concentration of 80w/v%); and
(iv) 150.48 g acrylamide (premixed in water at a concentration of 50w/v%) (both of (iii) and (iv) are acidified with about 16 g citric acid to pH 3.50); and
(v) 0.35 g Wako V50 initiator Wako (premixed with 56 g water), are dropped into the vessel over a period of 3 hours at a constant rate of addition. This mixture is then agitated for one further hour at 75°C. The polymerisation is completed by adding:
(vi) 1.40 g Wako V50 terminator (premixed with 56 g water).
The mixture is then agitated over a period of 3 hours at 75°C. Finally, the solution is filtered.

The resultant viscous solution showed a molar weight of 710,000 Da. (determined by GPC), a solids content of 20.9% and a pH value of 2.76. Residual acrylamide monomers could be detected in a range of 0.001 g / 100 g solution.

### Example 2 - Synthesis of a copolymer of acrylamide and DMA3MeCl (1:1 ratio)

The polymerisation reaction is carried out as described in example 1, but uses different amounts of ingredients.
(i) 787 g water.
(ii) 0.13 g Trilon C (premixed in water at a concentration of 40w/v%).
(iii) 228.53 g DMA3MeCl (premixed in water at a concentration of 80w/v%).
(iv) 134.36 g acrylamide (premixed in water at a concentration of 50w/v%).
(v) 1.25 g Wako V50 initiator (premixed with 50 g water).
(vi) 1.25 g Wako V50 terminator (premixed with 56 g water).

The resultant slightly viscous solution showed a molar weight of 210,000 Da. (determined by GPC).

### Example 3 - Synthesis of a copolymer of acrylamide and DMA3MeCl (5:1 ratio)

The polymerisation reaction is carried out as described in example 1, but uses different amounts of ingredients.
(i) 716 g water.
(ii) 0.32 g Trilon C (premixed in water at a concentration of 40w/v%).
(iii) 110.14 g DMA3MeCl (premixed in water at a concentration of 80w/v%).
(iv) 323.78 g acrylamide (premixed in water at a concentration of 50w/v%).
(v) 0.31 g Wako V50 initiator (premixed with 50g water).
(vii) 1.25 g Wako V50 terminator (premixed with 56 g water).

The resultant slightly viscous solution showed a molar weight of 230,000 Da. (determined by GPC).

### Example 4 - Synthesis of a copolymer of acrylamide and DMA3MeCl (5:1 ratio)

The polymerisation reaction is carried out as described in example 3, except that (v) 1.25 g Wako V50 initiator (premixed with 50 g water) was used.

The resultant slightly viscous solution showed a molar weight of 370,000 Da. (determined by GPC).

### Example 5 - Synthesis of a copolymer of acrylamide and DMA3MeCl (5:1 ratio)

The polymerisation reaction is carried out as described in example 3, except that (v) 2.50 g Wako V50 initiator (premixed with 50 g water) was used.

The resultant slightly viscous solution showed a molar weight of 230,000 Da. (determined by GPC).

### Example 6 - Synthesis of a copolymer of acrylamide and DMA3MeCl (24:1 ratio)

The polymerisation was carried out as described in example 1, except that different amounts of ingredients are used.
(i) 823 g water.
(ii) 0.54 g Trilon C (premixed in water at a concentration of 40w/v%).
(iii) 38.19 g DMA3MeCl (premixed in water at a concentration of 80w/v%).
(iv) 538.9 g acrylamide (premixed in water at a concentration of 50w/v%).
(v) 1.13 g Wako V50 initiator (premixed with 50g water).
(vi) 1.50 g Wako V50 terminator (premixed with 56 g water).

The resultant slightly viscous solution showed a molar weight of 780,000 Da. (determined by GPC).

### Example 7

The following perfume accords A, B and C are suitable for use in the present invention. Amounts given below are by weight of the perfume accord.

### Example 7 - perfume accord A

| **PRM trade name** | **PRM chemical name** | **Amount** |
|---|---|---|
| Damascone beta^{TM} | 2-buten-1-one, 1-(2,6,6-trimethyl-1-cyclohexen-1-yl)- | 1% |
| Dynascone 10^{TM} | 4-Penten-1-one, 1-(5,5-dimethyl-1-cyclohexen-1-yl)- | 5% |
| | Ethyl 2 Methyl Butyrate | 6% |
| Eugenol | 4-hydroxy-3-methoxy-1-allylbenzene | 1% |
| Cyclacet^{TM} | Tricyclo decenyl acetate | 3% |
| Cyclaprop^{TM} | Tricycle decenyl propionate | 6% |
| Ionone beta^{TM} | 2-(2,6,6-Trimethyl-1-cyclohexen-1-yl) -3-buten-2- | 8% |
| | one | |
| Nectaryl™ | 2-(2-(4-Methyl-3-cyclohexen-1-yl)propyl) cyclopentanone | 50% |
| Triplal™ | 3-cyclohexene-1-carboxaldehyde, dimethyl | 10% |
| Verdox™ | Ortho tertiary butyl cyclohexanyl acetate | 10% |

Perfume accord A is an example of a fruity perfume accord.

### Example 7 - perfume accord B

| **PRM trade name** | **PRM chemical name** | **Amount** |
|---|---|---|
| Ally amyl glycolate^{TM} | Glycolic acid, 2 -pentyloxy:allyl ester | 5% |
| Damascone beta^{TM} | 2-buten-1-one, 1-(2,6,6-trirnethyl-1-cyclohexen-16yl)- | 2% |
| Dynascone 10^{TM} | 4-Penten-1-one, 1-(5,5-dimethyl-1-cyclohexen-16yl)- | 5% |
| Hedione^{TM} | Cyclopentaneacetic acid, 3-oxo-2-pentyl- methyl ester | 25% |
| Iso cyclo citral | 3-cyclohexene-1-carboxaldehyde, 2,4,6-trimethyl | 5% |
| Lilial^{TM} | 2-Methyl-3-(4-tert-butylphenyl)propanal | 48% |
| Rose oxide | Methyl iso butenyl tetrahydro pyran | 5% |
| Triplal^{TM} | 3-cyclohexene-1-carboxaldehyde, dimethyl | 5% |

Perfume accord B is an example of a floral green perfume accord.

### Example 7 - perfume accord C

| **PRM trade name** | **PRM chemical name** | **Amount** |
|---|---|---|
| Hedione^{TM} | Cyclopentaneacetic acid, 3-oxo-2-pentyl- methyl ester | 30% |
| Isoraldeine 70^{TM} | Gamma-methylionone | 30% |
| Dodecanal | Lauric Aldehyde | 1% |
| Lilial^{TM} | 2-Methyl-3-(4-tert-butylphenyl)propanal | 30% |
| | Methyl Nonyl Acetaldehyde | 1% |
| Triplal^{TM} | 3-cyclohexene-1-carboxaldehyde, dimethyl | 5% |
| | Undecylenic Aldehyde | 3% |

Perfume accord C is an example of a floral aldehydic perfume accord.

### Example 8 - process for preparing an encapsulated perfume particle

The perfume accords of example 7 undergo the following process to obtain perfume particles that are suitable for use in the present invention.

Zeolite 13x is passed through a Schuggi mixer, wherein the perfume accord (any one of the perfume accords of example 7) is sprayed onto the zeolite 13x to obtain perfume-loaded zeolite 13x comprising 85% zeolite 13x and 15% perfume accord. The Schuggi mixer is operated at 2,000rpm to 4,000 rpm. Liquid nitrogen is used to control the build up of heat that occurs during this perfume-loading step, which is carried out at a temperature of below 40°C.

A 20wt% solution of cationic polyacrylamide (any one of the polymers of examples 1-6) is diluted in water to obtain a 2.9wt% solution. The perfumed zeolite described above is added to this solution resulting in a suspension (35wt% perfumed zeolite, 1.8wt% polymer 63.2wt% water). The suspension is stirred for 15 minutes. External cooling (water jacket) is provided, to keep the suspension temperature below 20°C.

A suspension of starch (33w/v% in water) is added to the suspension described above to form an encapsulation mixture comprising 10.8wt% starch, 23.5wt% perfume-loaded zeolite 13x, 1.2% cationic polymer and 64.5wt% water. This is carried out in a batch container. The time of this step is 2 minutes and the temperature is kept below 20°C by using a water jacket.

The encapsulation mixture is fed continuously to a buffer tank, from where it is spray dried. The encapsulation mixture is pumped into a Production Minor using a peristaltic pump and is then spray dried to obtain perfume particles. The rotary atomiser tip speed was 151.8 m/s (29,000rpm of a 10cm diameter atomiser). The inlet temperature of the spray-drying tower is 170°C and the outlet temperature of the spray-drying tower is 105°C.

### Example 9 - laundry detergent compositions

The perfume particles of example 8 are incorporated into the following solid laundry detergent composition, which are suitable for use in the present invention. Amounts given below are by weight of the composition.

| **Ingredient** | **A** | **B** | **C** | **D** | **E** |
|---|---|---|---|---|---|
| Perfume particle according to example 8 | 3% | 2% | 1% | 3% | 2% |
| Sodium linear _{C11-13} alkylbenzene sulphonate | 15% | 18% | 15% | 11% | 10% |
| R₂N⁺(CH₃)₂(C₂H₄OH), wherein R₂ = C₁₂-C₁₄ alkyl group | 0.6% | | 0.5% | 0.6% | |
| Sodium C₁₂₋₁₈ linear alkyl sulphate condensed with an average of 3 to 5 moles of ethylene oxide per mole of alkyl sulphate | | 2.0% | 0.8% | | |
| Mid chain methyl branched sodium C₁₂₋₁₈ linear alkyl sulphate | | | | 1.4% | |
| Sodium linear C₁₂₋₁₈ linear alkyl sulphate | | | | 0.7% | |
| Sodium tripolyphoshate (anhydrous weight given) | 25% | 22% | 30% | | |
| Citric acid | | | | 2.5% | 2.0% |
| Sodium carboxymethyl cellulose | 0.3% | 0.2% | | 0.2% | 0.2% |
| Hydrophobically modified (e.g. ester modified) cellulose | | | | 0.8% | 0.7% |
| Sodium polyacrylate polymer having a weight average molecular weight of from 3,000 to 5,000 | | 0.5% | 0.8% | | |
| Copolymer of maleic/acrylic acid, having a weight average molecular weight of from 50,000 to 90,000, wherein the ratio of maleic to acrylic acid is from 1:3 to 1:4 | | | | 1.4% | 1.5% |
| Sulphated or sulphonated bis((C₂H₅O)(C₂H₄O)ₙ)(CH₃)N⁺CₓH₂ₓN⁺( CH₃)bis(C₂H₅O)(C₂H₄O)ₙ), wherein n= from 20 to 30 and x = from 3 to 8 | | 1.5% | 1.0% | | 1.0% |
| Diethylene triamine pentaacetic acid | 0.2% | 0.3% | 0.3% | | |
| Diethylene triamine pentaacetic acid | | | | 0.2% | 0.3% |
| Proteolytic enzyme having an enzyme activity of from 15mg/g to 70mg/g | 0.5% | 0.4% | 0.5% | 0.1% | 0.15% |
| Amylolytic enzyme having an enzyme activity of from 25mg/g to 50mg/g | 0.2% | 0.3% | 0.3% | 0.2% | 0.1% |
| Anhydrous sodium perborate monohydrate | 5% | 4% | 5% | | |
| Sodium percarbonate | | | | 6% | 8% |
| Magnesium sulphate | | | | 0.4% | 0.3% |
| Nonanoyl oxybenzene sulphonate | 2% | 1.5% | 1.7% | | |
| Tetraacetylethylenediamine | 0.6% | 0.8% | 0.5% | 1.2% | 1.5% |
| Brightener | 0.1% | 0.1% | 0.1% | 0.04% | 0.03% |
| Sodium carbonate | 25% | 22% | 20% | 28% | 20% |
| Sodium sulphate | 14% | 14% | 7% | 12% | 15% |
| Zeolite A | 1% | 1.5% | 2% | 20% | 18% |
| Sodium silicate (2.0R) | 0.8% | 1% | 1% | | |
| Crystalline layered silicate | | | | 3% | 3.5% |
| Photobleach | 0.005% | 0.004% | 0.005% | 0.001% | 0.002% |
| Montmorillonite clay | | | 4% | | 6% |
| Polyethyleneoxide having a weight average molecular weight of from 100,000 to 1,000,000 | | | 1% | | 2% |
| Perfume spray-on | | 0.5% | 0.3% | | 0.3% |
| Starch encapsulated perfume accord | | | 0.2% | | 0.2% |
| Silicone based suds suppressor | | | | 0.05% | 0.06% |
| Miscellaneous and moisture | to 100% | to 100% | to 100% | to 100% | to 100% |

## Claims

1. A detergent auxiliary composition in particulate form, comprising:
(i) a liquid or liquefiable active component; and
(ii) a water-insoluble solid support component and
(iii) a water-soluble and/or water-dispersible encapsulating material; and
(iv) optionally one or more adjunct components,
**characterised in that** the composition further comprises
(v) a surface deposition enhancing cationic polymer,
wherein at least part of, preferably all of, the surface deposition enhancing cationic polymer is adsorbed onto the water-insoluble solid support component, and wherein the water-soluble and/or water dispersible encapsulating material encapsulates all of, the liquid or liquefiable active component, the water-insoluble solid support component and the surface deposition enhancing cationic polymer.

2. A composition according to claim 1, wherein the water-insoluble solid support component is porous.

3. A composition according to any preceding claim, wherein the water-insoluble solid support component is an aluminosilicate, preferably a zeolite.

4. A composition according to any preceding claim, wherein the water-insoluble solid support component has a negative surface charge, preferably the solid support component comprises an oxide outer surface.

5. A composition according to any preceding claim, wherein the liquid or liquefiable active component is a perfume.

6. A composition according to any preceding claim, wherein the water-soluble and/or water dispersible encapsulating material comprises a polysaccharide, preferably a starch, and optionally a plasticiser.

7. A composition according to any preceding claim, wherein the surface deposition enhancing cationic polymer is water-soluble and/or water-dispersible, preferably water-soluble.

8. A composition according to any preceding claim, wherein the composition comprises from 1.2wt% to 10wt% surface deposition enhancing cationic polymer.

9. A composition according to any preceding claim, wherein the surface deposition enhancing cationic polymer has a weight average molecular weight of from above 100,000 Da. to below 10,000,000 Da., preferably from 500,000 Da. to 2,000,000 Da..

10. A composition according to any preceding claim, wherein the surface deposition enhancing cationic polymer has an average degree of cationic substitution of from above 2% to 70%, preferably from 40% to 60%.

11. A composition according to any preceding claim, wherein the surface deposition enhancing cationic polymer is a co polymer of acrylamide and a methyl chloride quaternary salt of dimethylaminoethyl acrylate, the surface deposition enhancing cationic polymer having the general formula: wherein n and m independently are numbers in the range of from 100 to 100,000, preferably from 800 to 3400, and the molar ratio of n:m is in the range of from 4:1 to 3:7, preferably from 3:2 to 2:3.

12. A composition according to any preceding claim, wherein the zeta potential of the composition is more neutral than -30mV, preferably more neutral than -20mV.

13. A composition according to any preceding claim, wherein the composition has a mean particle size of from 5 micrometers to 200 micrometers, preferably from 10 to 50 micrometers, and preferably no more than 10wt% of the composition has a particle size less than 5 micrometers and preferably no more than 10wt% of the composition has a particle size greater than 80 micrometers.

14. A method of making a composition according to any preceding claim, the method comprising the steps of:
(i) contacting a water-insoluble solid support component with a liquid or liquefiable active component to form a first mixture; and
(ii) contacting the first mixture obtained in step (i) with a surface deposition enhancing cationic polymer to form a second mixture; and
(iii) contacting the second mixture obtained in step (ii) with a water-soluble and/or water-dispersible encapsulating material to form a composition; and
(iv) optionally, drying the composition of step (iii),
wherein step (ii) occurs subsequent to step (i) and prior to steps (iii) and (iv).

15. A method according to claim 14, wherein in step (ii), the surface deposition enhancing polymer is present in an aqueous mixture at a concentration of from 0.3g/l to 50g/l.

16. A method according to claims 14-15, wherein in step (ii), the water-insoluble solid support component is present in an aqueous mixture at a concentration of from 7g/l to 7,000g/l.

17. A method according to claims 14-16, wherein in step (iv) the composition of step (iii) is spray-dried.

18. A laundry detergent composition comprising a detergent auxiliary composition according to any of claims 1-13 and optionally one or more adjunct components.

## Patentansprüche

1. Reinigungshilfsmittelzusammensetzung in Teilchenform, umfassend:
(I) einen flüssigen oder verflüssigbaren Wirkbestandteil und
(II) einen wasserunlöslichen festen Trägerbestandteil und
(III) ein wasserlösliches und/oder wasserdispergierbares Verkapselungsmaterial und
(IV) wahlweise einen oder mehrere Zusatzbestandteile,
**dadurch gekennzeichnet, dass** die Zusammensetzung ferner Folgendes umfasst
(V) ein die Oberflächenanlagerung verbesserndes kationisches Polymer,
wobei mindestens ein Teil, vorzugsweise die Gesamtheit des die Oberflächenanlagerung verbessernden kationischen Polymer an den wasserunlöslichen festen Trägerbestandteil angelagert wird und wobei das wasserlösliche und/oder wasserdispergierbare Verkapselungsmaterial den gesamten flüssigen oder verflüssigbaren Wirkbestandteil, den gesamten wasserunlöslichen festen Trägerbestandteil und das gesamte die Oberflächenanlagerung verbessernde kationische Polymer einkapselt.

2. Zusammensetzung nach Anspruch 1, wobei der wasserunlösliche feste Trägerbestandteil porös ist.

3. Zusammensetzung nach einem der vorstehenden Ansprüche, wobei der wasserunlösliche feste Trägerbestandteil ein Alumosilicat, vorzugsweise ein Zeolith, ist.

4. Zusammensetzung nach einem der vorstehenden Ansprüche, wobei der wasserunlösliche feste Trägerbestandteil eine negative Oberflächenladung aufweist, wobei der feste Trägerbestandteil vorzugsweise eine Oxid-Außenoberfläche umfasst.

5. Zusammensetzung nach einem der vorstehenden Ansprüche, wobei der flüssige oder verflüssigbare Wirkbestandteil ein Duftstoff ist.

6. Zusammensetzung nach einem der vorstehenden Ansprüche, wobei das wasserlösliche und/oder wasserdispergierbare Verkapselungsmaterial ein Polysaccharid, vorzugsweise eine Stärke, und wahlweise einen Weichmacher umfasst.

7. Zusammensetzung nach einem der vorstehenden Ansprüche, wobei das die Oberflächenanlagerung verbessernde kationische Polymer wasserlöslich und/ oder wasserdispergierbar, vorzugsweise wasserlöslich, ist.

8. Zusammensetzung nach einem der vorstehenden Ansprüche, wobei die Zusammensetzung 1,2 Gew.-% bis 10 Gew.-% die Oberflächenanlagerung verbesserndes kationisches Polymer umfasst.

9. Zusammensetzung nach einem der vorstehenden Ansprüche, wobei das die Oberflächenanlagerung verbessernde kationische Polymer ein Molekulargewicht-Gewichtsmittel von über 100.000 Da bis unter 10.000.000 Da, vorzugsweise von 500.000 Da bis 2.000.000 Da, aufweist.

10. Zusammensetzung nach einem der vorstehenden Ansprüche, wobei das die Oberflächenanlagerung verbessernde kationische Polymer einen durchschnittlichen Grad der kationischen Substitution von über 2 % bis 70 %, vorzugsweise von 40 % bis 60 % aufweist.

11. Zusammensetzung nach einem der vorstehenden Ansprüche, wobei das die Oberflächenanlagerung verbessernde kationische Polymer ein Copolymer von Acrylamid und einem quartären Methylchloridsalz von Dimethylaminoethylacrylat ist, wobei das die Oberflächenanlagerung verbessernde kationische Polymer die folgende allgemeine Formel aufweist: wobei n und m unabhängig voneinander Zahlen im Bereich von 100 bis 100.000, vorzugsweise von 800 bis 3400 sind und das Molverhältnis von n:m im Bereich von 4:1 bis 3:7, vorzugsweise von 3:2 bis 2:3 liegt.

12. Zusammensetzung nach einem der vorstehenden Ansprüche, wobei das Zeta-Potential der Zusammensetzung neutraler als -30 mV, vorzugsweise neutraler als -20 mV ist.

13. Zusammensetzung nach einem der vorstehenden Ansprüche, wobei die Zusammensetzung eine mittlere Teilchengröße von 5 Mikrometer bis 200 Mikrometer, vorzugsweise von 10 bis 50 Mikrometer aufweist und vorzugsweise nicht mehr als 10 Gew.-% der Zusammensetzung eine Teilchengröße von weniger als 5 Mikrometer aufweisen und vorzugsweise nicht mehr als 10 Gew.-% der Zusammensetzung eine Teilchengröße von mehr als 80 Mikrometer aufweisen.

14. Verfahren zum Herstellen einer Zusammensetzung nach einem der vorstehenden Ansprüche, wobei das Verfahren die folgenden Schritte umfasst:
(I) Inkontaktbringen eines wasserunlöslichen festen Trägerbestandteils mit einem flüssigen oder verflüssigbaren Wirkbestandteil, um eine erste Mischung zu bilden, und
(II) Inkontaktbringen der in Schritt (I) hergestellten ersten Mischung mit einem die Oberflächenanlagerung verbessernden kationischen Polymer, um eine zweite Mischung zu bilden, und
(III) Inkontaktbringen der in Schritt (II) hergestellten zweiten Mischung mit einem wasserlöslichen und/oder wasserdispergierbaren Verkapselungsmaterial, um eine Zusammensetzung zu bilden, und
(IV) wahlweise Trocknen der Zusammensetzung von Schritt (III), wobei Schritt (II) nach Schritt (I) und vor den Schritten (III) und (IV) erfolgt.

15. Verfahren nach Anspruch 14, wobei in Schritt (II) das die Oberflächenanlagerung verbessernde Polymer in einer wässrigen Mischung in einer Konzentration von 0,3 g/l bis 50 g/l vorliegt.

16. Verfahren nach Anspruch 14 bis 15, wobei in Schritt (II) der wasserunlösliche feste Trägerbestandteil in einer wässrigen Mischung in einer Konzentration von 7 g/l bis 7.000 g/l vorliegt.

17. Verfahren nach Anspruch 14 bis 16, wobei in Schritt (IV) die Zusammensetzung von Schritt (III) sprühgetrocknet wird.

18. Wäschewaschmittelzusammensetzung, umfassend eine Reinigungshilfsmittelzusammensetzung nach einem der Ansprüche 1 bis 13 und wahlweise einen oder mehrere Zusatzbestandteile.

## Revendications

1. Composition auxiliaire détergente sous forme particulaire, comprenant :
(i) un composant actif liquide ou liquéfiable ; et
(ii) un composant support solide insoluble dans l'eau et
(iii) un matériau d'encapsulation hydrosoluble et/ou hydrodispersible ; et
(iv) facultativement un ou plusieurs composants additifs,
**caractérisée en ce que** la composition comprend en outre
(v) un polymère cationique améliorant le dépôt en surface,
dans laquelle au moins une partie, de préférence la totalité, du polymère cationique améliorant le dépôt en surface est adsorbée sur le composant support solide insoluble dans l'eau, et dans laquelle le matériau d'encapsulation hydrosoluble et/ou hydrodispersible encapsule la totalité du composant actif liquide ou liquéfiable, du composant support solide insoluble dans l'eau et du polymère cationique améliorant le dépôt en surface.

2. Composition selon la revendication 1, dans laquelle le composant support solide insoluble dans l'eau est poreux.

3. Composition selon l'une quelconque des revendications précédentes, dans laquelle le composant support solide insoluble dans l'eau est un aluminosilicate, de préférence une zéolite.

4. Composition selon l'une quelconque des revendications précédentes, dans laquelle le composant support solide insoluble dans l'eau a une charge de surface négative, de préférence le composant support solide comprend une surface externe d'oxyde.

5. Composition selon l'une quelconque des revendications précédentes, dans laquelle le composant actif liquide ou liquéfiable est un parfum.

6. Composition selon l'une quelconque des revendications précédentes, dans laquelle le matériau d'encapsulation hydrosoluble et/ou hydrodispersible comprend un polysaccharide, de préférence un amidon, et facultativement un plastifiant.

7. Composition selon l'une quelconque des revendications précédentes, dans laquelle le polymère cationique améliorant le dépôt en surface est hydrosoluble et/ou hydrodispersible, de préférence hydrosoluble.

8. Composition selon l'une quelconque des revendications précédentes, où la composition comprend de 1,2 % en poids à 10 % en poids de polymère cationique améliorant le dépôt en surface.

9. Composition selon l'une quelconque des revendications précédentes, dans laquelle le polymère cationique améliorant le dépôt en surface a une masse moléculaire moyenne en poids allant de plus de 100 000 Da à moins de 10 000 000 Da, de préférence de 500 000 Da à 2 000 000 Da.

10. Composition selon l'une quelconque des revendications précédentes, dans laquelle le polymère cationique améliorant le dépôt en surface a un degré moyen de substitution cationique allant de plus de 2 % à 70 %, de préférence de 40 % à 60 %.

11. Composition selon l'une quelconque des revendications précédentes, dans laquelle le polymère cationique améliorant le dépôt en surface est un copolymère d'acrylamide et un sel quaternaire chlorure de méthyle d'acrylate de diméthylaminoéthyle, le polymère cationique améliorant le dépôt en surface étant de formule générale : dans laquelle n et m sont indépendamment des nombres dans l'intervalle allant de 100 à 100 000, de préférence de 800 à 3400, et le rapport molaire de n:m est dans l'intervalle allant de 4:1 à 3:7, de préférence de 3:2 à 2:3.

12. Composition selon l'une quelconque des revendications précédentes, dans laquelle le potentiel zêta de la composition est plus neutre que -30 mV, de préférence plus neutre que -20 mV.

13. Composition selon l'une quelconque des revendications précédentes, où la composition a une taille moyenne des particules allant de 5 micromètres à 200 micromètres, de préférence de 10 à 50 micromètres, et de préférence pas plus de 10 % en poids de la composition a une taille des particules inférieure à 5 micromètres et de préférence pas plus de 10 % en poids de la composition a une taille des particules supérieure à 80 micromètres.

14. Procédé de fabrication d'une composition selon l'une quelconque des revendications précédentes, le procédé comprenant les étapes consistant à :
(i) mettre en contact un composant support solide insoluble dans l'eau avec un composant actif liquide ou liquéfiable de façon à former un premier mélange ; et
(ii) mettre en contact le premier mélange obtenu dans l'étape (i) avec un polymère cationique améliorant le dépôt en surface de façon à former un deuxième mélange ; et
(iii) mettre en contact le deuxième mélange obtenu dans l'étape (ii) avec un matériau d'encapsulation hydrosoluble et/ou hydrodispersible de façon à former une composition ; et
(iv) facultativement, sécher la composition de l'étape (iii),
dans lequel l'étape (ii) se produit après l'étape (i) et avant les étapes (iii) et (iv).

15. Procédé selon la revendication 14, dans lequel dans l'étape (ii), le polymère améliorant le dépôt en surface est présent dans un mélange aqueux à une concentration allant de 0,3 g/L à 50 g/L.

16. Procédé selon la revendication 14 à 15, dans lequel dans l'étape (ii), le composant support solide insoluble dans l'eau est présent dans un mélange aqueux à une concentration allant de 7 g/L à 7000 g/L.

17. Procédé selon les revendications 14 à 16, dans lequel dans l'étape (iv), la composition de l'étape (iii) est séchée par atomisation.

18. Composition détergente pour le lavage du linge comprenant une composition auxiliaire détergente selon l'une quelconque des revendications 1 à 13 et facultativement un ou plusieurs composants additifs.
